

March 15, 1932.

W. S. BAYLIS

1,849,654

METHOD OF RECLAMING USED LUBRICATING OILS

Filed Oct. 14, 1926



## UNITED STATES PATENT OFFICE

WALTER S. BAYLIS, OF LOS ANGELES, CALIFORNIA, ASSIGNOR, BY MESNE ASSIGNMENTS, TO FILTROL COMPANY OF CALIFORNIA, A CORPORATION OF CALIFORNIA

## METHOD OF RECLAIMING USED LUBRICATING OILS

Application filed October 14, 1926. Serial No. 141,588.

My invention relates to oil refining processes, and it consists of a process of reclaiming used lubricating oil.

It is well known that lubricating oil loses its lubricating qualities by reason of its being impregnated with colloidal carbon, organic and inorganic acids, foreign matter and other impurities such as gasoline.

It is an object of my invention to provide a reclaiming process for treating used lubricating oil whereby the undesirable substances may be removed and the oil thus made suitable for reuse.

It is another object of this invention to provide a reclaiming process for treating used lubricating oil in which the used lubricating oil is mixed with an adsorptive material which adsorbs all the impurities of the oil with the exception of the very light distillates; the adsorptive material carrying the impurities afterwards being separated from the lubricating oil by filtration.

It is another object of my invention to provide a process of this character in which the lubricating oil is subjected to the action of hot vapors in order to evaporate the light distillates therefrom and to reduce the oil to a desired viscosity.

I have found that by adding silicate of soda to the used lubricating oil and adsorptive material, the fatty or organic acids are readily collected and adsorbed by the adsorptive material.

It is, therefore, an object of my invention to provide a process for recovering used lubricating oil in which silicate of soda or some other agglomerating agent is mixed with the oil and adsorptive material.

It is also an object of my invention to provide a process of this character in which the oil is distilled under a high vacuum to prevent oxidization and cracking of the oil.

Other objects and advantages of the invention will be made evident hereinafter.

Referring to the drawings in which an apparatus for conducting my invention is shown,

1 is a mixer, 2 is a pressure pump, 3 is a primary filter press, 4 is a still, 5 is a liquid trap, 6 is a condenser, 7 is a vacuum pump,

8 is an expansion vessel, 9 is a pressure pump, 10 is a secondary filter and 11 is an oil cooler.

The mixer 1 consists of a shell 12 having a conical bottom 3 and which is open at the top end thereof. Surrounding the shell 12 is a jacket 14 providing a heating chamber 15 which has pipes 16 connected thereto by means of which a suitable heating medium such as steam is supplied to and taken from the chamber 15, this heating medium being for the purpose of heating the interior of the mixer 1. Mixing paddles 18 are positioned in the mixer 1, being rigidly secured on a shaft 19 which is supported by bearings 17. The shaft 19 is adapted to be driven by gears 20 which are secured at the upper end of the shaft 19. Used lubricating oil is supplied to the mixer 1 by means of an oil pipe 13. This used lubricating oil contains colloidal carbon, foreign matter, acids and other impurities such as distillates which have been added thereto during its use.

A small percentage of adsorptive material is added to the oil in the mixer 1 and is thoroughly mixed therewith by means of the mixing paddles 18 which are operated when the shaft 19 rotates. Also, a small percentage of agglomerating agent is added to the mixture of oil and adsorptive material by means of a pipe 21 and is also mixed with the oil. The temperature of the mixture in the mixer 1 is raised to about 220° F. The adsorptive material during the time that it is being mixed with the oil adsorbs the foreign material, colloidal carbon and other impurities with which the lubricating oil is impregnated. The agglomerating agent operates to collect all of the fatty or organic acids so that they may be readily adsorbed by the adsorptive material. All of the organic and inorganic acids are thus removed from the lubricating oil and the lubricating oil is entirely neutralized.

When the mixing has continued a sufficient length of time to permit all of the undesirable substances to be adsorbed by the adsorptive material, the mixture is removed to the primary filter press 3. A pipe 24 extends from the conical bottom 3 of the mixer 1 to the pressure pump 2, this pipe 24 having a

valve 22 which is closed while the mixing is being carried on in the mixer. Extending from the pressure pump 2 to the primary filter press 3 is a pipe 23. The valve 22 is opened (when the mixing is complete) and the pressure pump 2 is set into operation to pump the mixture from the mixer 1 into the filter press 3.

The filter press 3 is of standard construction and consists of a shell 31 providing a chamber 32. Placed in the chamber 32 is a plurality of screens or filter bags 33, the interior of which have pipes 34 connected thereto which join to an outlet manifold 35. The mixture passes into the chamber 32 of the filter press 3. The oil passes into the interior of the screens or filter bags 33 and passes through the pipes 34 into the manifold 35. The adsorptive material carrying the undesirable substances of the lubricating oil is too coarse to pass through the bags 33 and therefore collects in cakes 37 on the exteriors of the bags, as shown in the drawing. This operation removes all the impurities or moisture and leaves a clear oil containing only the very light distillates.

The filtered oil and light distillates are carried to the still 4 by means of a pipe 38 having a valve 39 which connects with the manifold 35 and the still 4. The still 4 consists of a shell 41 having a conical bottom 42 and a tight top 43. The pipe 38 connects with the interior of the still 4 through the top 43. Mixing paddles 44 are supported in the shell 41 by a shaft 45 which is rotatable in bearings 46. The shaft 45 extends from the top 43 of the still 4 and is adapted to be operated by gearing 47. The shell 41 is provided with a jacket 48 to which pipes 49 connect for supplying a heating medium to a chamber 51 provided between the jacket and shell for the purpose of heating the interior of the still 4.

The clear oil containing the light distillates is mixed with a small percentage of fresh adsorptive material in the still 4 by the operation of the mixing paddles 44, this adsorptive material being introduced into the still 4 through an opening closed by a tight cover 52. A high vacuum is placed upon the interior of the still 4 by means of a pipe 53 which connects to the interior of the still 4 through the tight top 43 thereof.

During the mixing of the clear oil and the fresh adsorptive material in the still 4, steam is introduced into the still by means of a pipe 54 having a valve 55, said pipe 54 extending through the conical bottom 42 of the still. This steam passes upwardly through the mixture of clear oil and adsorptive material and heats the oil to the extent that the light distillates are distilled therefrom.

The vapor composed of steam and light distillate vapors is drawn through the pipe 53 by the vacuum created by the vacuum

pump 7. The pipe 53 connects to the liquid trap 5. This liquid trap 5 consists of a shell 57 having a baffle plate 58. The vapor is introduced into the liquid trap 5 and passes around the baffle plate 58. The vapor is deprived of any particles of liquid which it may carry during its passage through the liquid trap 5. A pipe 61 connects the interior of the liquid trap 5 with the condenser 6.

The condenser 6 consists of a shell 62, the ends of which are closed by tight covers 63. Intermediate heads 64 are secured inside the shell 62 between which pipes 65 are extended. Pipes 67 are connected to the space between the head 64 and around the pipes 65 for introducing into and taking cooling medium from this space. The vapor is introduced into a space at the upper end of the condenser 6 and is passed through the tubes 65 into a space at the lower end of the condenser 6. Any portions of the vapor having a higher boiling point than water are condensed in the condenser 6 and may be delivered therefrom by a pipe 68 having a valve 69 which is connected with the lower chamber of the condenser.

A pipe 71 connects the lower chamber of the condenser 6 with the vacuum pump 7 and the vapors are drawn by the vacuum pump 7 from the condenser 6 through this pipe 71. A pipe 73 connects the vacuum pump 7 with an expansion vessel 8 through which pipe 73 the vapors are passed.

The expansion vessel 8 consists of a shell 81 having tight ends 82. Intermediate heads 83 are secured in the shell 80 between which heads pipes 84 extend. A cooling medium is supplied to and taken from a space around the pipes 84 and between the heads 83 by pipes 86. The vapor passes from the pipe 73 into an upper chamber of the expansion vessel 8 and passes through the pipes 84 into a lower chamber of the expansion vessel 8. During the passage of the vapor through the expansion vessel 8, the condensable constituents thereof are condensed and the permanent gases are taken from the lower chamber by means of a pipe 87, these gases being conducted to tanks or being expelled to the atmosphere. The condensates are taken from the lower chamber of the expansion vessel 8 by means of a pipe 88 having a valve 89. The condensate consists essentially of water and light distillate and is conducted to suitable tanks where the distillate may be separated from the water by gravity, the distillate forming a valuable by-product.

The clear oil in the still 4 is bleached and the light distillates are distilled therefrom. By carrying on this operation of distillation under a high vacuum there will be no oxidizing or cracking of the lubricating oil which, of course, would cause odorization. After the oil has been subjected to this action for the proper length of time it is taken from the

still 4 by the pressure pump 9 through a pipe 91 which connects to the still 4 through the conical bottom 42 thereof and which has a valve 92. The pump 9 forces the oil which has been mixed with fresh adsorptive material through a pipe 94 to the secondary filter press 10.

The secondary filter press 10 consists of a shell 101 with which the pipe 94 connects. The shell 101 provides a chamber 102 in which a plurality of filter bags 103 are placed. The interiors of these filter bags 103 have pipes 104 connected therewith, which pipes 104 join to a header 106 of the secondary filter press 10 situated on the outside of the shell 101. The clear oil is forced through the bags 103 and passes through the pipes 104 into the header 106, the adsorptive material collecting in a cake on the outside of each of the bags 103, as indicated at 108. The clear oil is separated from the adsorptive material in the filter press 10 and is conducted therefrom through a pipe 112, which connects to the header 106 and has a valve 113, to an oil cooler 11.

The oil cooler 11 consists of a shell 115 providing a chamber in which a coil 116 is situated. A cooling medium is passed through the coil 116 for cooling the reclaimed lubricating oil to a normal temperature. The interior of the shell 115 is kept under a vacuum through a vacuum pipe 118 which connects to the pipe 53. The oil is cooled to normal temperature before it comes into contact with the air and is therefore stabilized and will not decompose and odorize. The cooled oil may be drawn from the cooler 11 by a pipe 119 having a valve 120.

The apparatus shown in the drawing comprises no part of my invention and is essentially standard equipment. The primary and secondary filters 3 and 10 are preferably Sweetland filters which have characteristics which make them very suitable for this use.

In carrying out my process I intend to use for the adsorptive material a special treated clay such as that known on the market as "Filtrol". Filtrol is an acid treated clay made by a process somewhat similar to that disclosed in U. S. Patent 1,897,113, granted to P. W. Prutzman on Nov. 15, 1921, and possesses adsorptive qualities and other characteristics which make it very valuable for this use. I intend to use from 5% to 20% of spent or once used "Filtrol" in the mixer 1, such as that which is taken from the secondary filter 10, and to use from 5% to 15% of fresh "Filtrol" in the still 4. The percentages of "used" and "fresh" "Filtrol" vary within the above-mentioned amounts, depending upon (1) the condition of the used oil and (2) the desired degree of refinement. This practice is quite economical and assures a complete adsorption of the impurities.

As an agglomerating agent I purpose to use

from 2% to 10% of a silicate of soda solution, since it is very effective in collecting the organic or fatty acids and therefore in assisting the Filtrol in its adsorption of impurities.

From the foregoing description it is obvious that my process treats and converts used lubricating oil into a valuable product which may be again used for lubricating purposes. The reclaimed oil produced by my invention is in some instances better than the oil in its original condition. It is quite obvious that the process of my invention is really a re-distillation process and therefore the lubricating oil is refined to a greater extent. Any viscosity of oil may be had, this depending upon the time that the clear oil is treated in the still 4. The longer the oil is treated, the more viscous it becomes.

I claim as my invention:

1. A process for reclaiming used lubricating oil comprising: mixing a used lubricating oil with an acid-activated clay material and an agglomerating agent in the form of silicate of soda for adsorbing impurities from said oil; filtering said clay which carries said impurities from said oil; and distilling the light distillates from said oil.

2. A process for reclaiming used lubricating oil comprising: mixing a used lubricating oil with an adsorptive material in the form of an acid-activated clay and an agglomerating agent in the form of silicate of soda for adsorbing impurities from said oil; filtering said adsorptive material which carries said impurities from said oil; and distilling the light distillates from said oil.

3. A process for reclaiming used lubricating oil comprising: mixing a used lubricating oil with an adsorptive material in the form of an acid-activated clay and an agglomerating agent in the form of silicate of soda for adsorbing impurities from said oil; heating said oil during said mixing; filtering said adsorptive material which carries said impurities from said oil; and distilling the light distillates from said oil.

4. A process for reclaiming used lubricating oil comprising: mixing a used lubricating oil with an adsorptive material in the form of an acid-activated clay and an agglomerating agent in the form of silicate of soda for adsorbing impurities from said oil; filtering said adsorptive material which carries said impurities from said oil; mixing said oil with a fresh batch of acid-activated clay; distilling the light distillates from said mixture; and filtering said second batch of clay from said oil.

5. A process for reclaiming used lubricating oil comprising: mixing a used lubricating oil with an adsorptive material in the form of an acid-activated clay and an agglomerating agent in the form of silicate of soda for adsorbing impurities from said oil; heating

5 said oil during said mixing; filtering said adsorptive material which carries said impurities from said oil; mixing said oil with a second adsorptive material; distilling the light distillates from said mixture; and filtering said second adsorptive material from said oil.

6. A process for reclaiming used lubricating oil, comprising: mixing a used lubricating oil with a previously used acid-activated clay and an agglomerating agent for adsorbing impurities from said oil; filtering said clay from said oil; mixing said oil with fresh acid-activated clay; distilling the light distillates from said mixture in order to restore the flash, fire and viscosity of that portion of the oil left in the still, while said mixture is agitated; and filtering said clay from said residual portion of the oil.

10 15 20 25 In testimony whereof, I have hereunto set my hand at Los Angeles, California, this 5th day of October, 1926.

WALTER S. BAYLIS.

30

35

40

45

50

55

60

65